

Dec. 1, 1925.

1,563,943

R. B. ADAMS ET AL

TOP PRESS ROLL FOR PAPER MAKING MACHINES

Filed Dec. 22, 1924



Inventors  
Raleigh B. Adams  
Frederick R. Woodward  
George A. Rockwell, *att'y.*  
by

Patented Dec. 1, 1925.

1,563,943

# UNITED STATES PATENT OFFICE.

RALEIGH B. ADAMS AND FREDERICK R. WOODWARD, OF NEWTON, MASSACHUSETTS,  
ASSIGNORS TO STOWE & WOODWARD COMPANY, OF NEWTON UPPER FALLS, MASSA-  
CHUSETTS, A CORPORATION OF MASSACHUSETTS.

## TOP PRESS ROLL FOR PAPER-MAKING MACHINES.

Application filed December 22, 1924. Serial No. 757,529.

To all whom it may concern:

Be it known that we, RALEIGH B. ADAMS and FREDERICK R. WOODWARD, both citizens of the United States, and both residents of Newton, in the county of Middlesex and Commonwealth of Massachusetts, have invented a new and useful Top Press Roll for Paper-Making Machines, of which the following is a specification.

10 In the ordinary machine for making paper there is usually a plurality of top press rolls and our invention is particularly useful when embodied in the first top press roll, the acting surface of which should be 15 resilient but such that the soft pulp will not stick to it.

Our object is to provide such a press roll having a porous active surface or periphery but the porosity is provided by holes in the 20 body itself of the roll.

We accomplish this object by compounding the rubber, and in this term we include rubber compound, with a chemical which is soluble in water so that when the roll is 25 finished and put into use on a paper machine the water, which is being squeezed out by the roll, dissolves out the minute particles of the chemical, leaving the acting surface porous and highly efficient for the prevention 30 of sticking, there being in fact holes or surface openings in the body itself, which give uniform action in the prevention of sticking.

The figure in the drawing represents a top 35 press roll in which the stippling A represents the holes or openings in the surface of the body of the roll.

Any suitable chemical may be used which is soluble in water but we prefer to use 40 sugar or common salt because these lend themselves better to proper mixture with the rubber or rubber compound and because they properly stand the vulcanizing conditions which are desirable in making these 45 rolls.

The process of making our roll, the process being a feature of our invention, consists 50 preferably in thoroughly mixing or compounding rubber or rubber compound with a chemical which is soluble in water, then preferably vulcanizing the compound to an iron core, then bringing the roll into contact with water as, for example, by squeezing out the water when the roll is in use in

a paper making machine, this squeezing or 55 other contact dissolving the minute particles of the chemical leaving the surface porous. We prefer to use, depending on circumstances, chemical to the extent of 10% to 50% of the amount of rubber used. 60

In compounding we make the soluble material of such fineness as to make the openings suitably small and its mixture with the rubber is sufficiently intimate to provide uniformity so that when the soluble material is dissolved out the holes are very numerous and uniformly dispersed. 65

Rolls of the character referred to are usually operated with a doctor pressed against them and in the past this doctor has had a 70 glazing action on the surface of the roll, as, for example, when it has been attempted to provide porosity by combining fibrous material with the rubber, this glazed condition tending to cause the paper to stick to the 75 rubber. With our roll however the doctor, acting with the water, tends to open the surface as the rubber wears and brings up more particles of soluble material to the action of the doctor and of the water and 80 thus the porous condition of the surface of the roll is maintained and consequently sticking of the paper to the roll is prevented.

What we claim is:

1. A top press roll whose surface comprises rubber and a chemical which is soluble in water.

2. A vulcanized top press roll whose surface comprises rubber and sodium chloride. 90

3. A top press roll whose surface comprises rubber and a chemical soluble in water, the chemical being from 10 to 50 per cent of the amount of rubber.

4. The process of making a top press roll 95 consisting in compounding rubber and a chemical which is soluble in water, then removing the chemical which is adjacent to the surface of the roll by the action of water and a doctor leaving the surface of the rubber porous, and then, according as the rubber wears, using the doctor and water to open up said surface and to bring up more particles of said chemical to the surface of the roll so as to be dissolved and thereby 100 retain the porous condition of the surface. 105

RALEIGH B. ADAMS.

FREDERICK R. WOODWARD.